

## UNITED STATES PATENT OFFICE.

LEE B. GREEN, OF LAKEWOOD, OHIO, ASSIGNOR TO THE BORDEN COMPANY, OF WARREN, OHIO, A CORPORATION OF OHIO.

## METHOD OF PREPARING SOLID FUELS FOR BURNING IN PULVERIZED FORM.

No Drawing.

Application filed November 20, 1926. Serial No. 149,799.

This invention relates to a method of preparing solid fuels, such as coal, for burning in pulverized form in burners of the type that are now known and used for burning pulverized coal.

In the art of burning pulverized fuels, such as coal, it is usual to pulverize the fuel and then introduce it into a blast of air in properly regulated amounts, the mixture of air and fuel being then conducted to a burner by which it is injected into a combustion chamber where the mixture is ignited and burned. In all known forms of apparatus, for this purpose, a supply of the pulverized fuel is maintained in a suitable storage reservoir from which it is gradually fed to the blast of air, and trouble has been experienced with this method of handling the fuel on account of its explosive nature when in pulverized form. In agitating the pulverized fuel preparatory to feeding it into the blast of air, a highly explosive mixture of air and fuel is produced, and sometimes trouble arises because of an explosion of this mixture in the fuel reservoir or in the apparatus conveying it to the burner, such explosions occurring frequently as a result of a back-fire from the burner or from a spark which might be created by the friction of parts comprising the feeding apparatus.

Heretofore, on account of the dangers which attended the use of pulverized fuel and the necessity for having skilled workmen to operate the equipment, it has been customary to confine the use of pulverized fuel to mills, power plants, and similar places, and it has been considered impracticable to use pulverized fuel in homes, apartment houses, and other places where relatively small apparatus would be required.

It is one of the objects of my invention to provide an improved method of preparing pulverized fuel that will permit the use of pulverized fuel burners in homes, apartment houses, and other places where only unskilled help is available and where only what may be termed fool-proof apparatus may be used.

A further object of the invention is to provide a method of preparing fuel for burning which will avoid the storage of pulverized fuel adjacent the burner and will

also avoid the objectionable dusty conditions that prevail around present installations for burning pulverized fuel.

55

A further object of the invention is to provide a method of preparing pulverized fuel that will permit the fuel to be maintained in the form of chunks or briquets until just prior to its introduction into the burner, thereby eliminating the danger that has heretofore attended the storage of fuel in the pulverized form.

Another object of the invention is to provide a system of preparing pulverized fuel that will permit the fuel to be initially prepared at points remote from the place of use, such as at mines or coal yards, and delivered to the point of use in the form of chunks, blocks, or briquets, which may be stored in a coal bin adjacent the point of use in much the same manner that ordinary coal is stored in homes and apartment houses.

70  
75  
Other objects of the invention and the features of novelty will be apparent from the following description wherein I describe what I now consider to be the preferred method of practicing the invention.

According to my preferred method of practicing my invention, I take ordinary coal, either hard or soft coal, and run it through a pulverizing machine in which it is reduced to a fineness that will be uniformly less than a predetermined size, such as a fineness that will pass through what is known as a 200 mesh screen. This reference to a specific fineness is mentioned merely by way of example, and as a matter of fact the fineness may be varied within wide limits. However, the largest particles must be of a fineness such that they can be carried into suspension and burned if they should be broken loose from the briquet without being reduced by the scraping or abrading means hereinafter referred to. This pulverized coal is then introduced into an ordinary briquetting machine, together with a suitable amount of binding material, such as coal tar, where these materials are thoroughly mixed and then compressed into blocks or briquets of any preferred size, and, for this purpose, I would recommend blocks 6" x 6" x 6" or 6" x 6" x 12". When soft coal is used, I prefer to subject the blocks, in the briquet-

85

90

95

100

ting operation, to a sufficient pressure that will tend to bring the oil in the fuel to the surface of the particles so that these particles will not have a dry, dusty nature. In any 5 event, the pressure preferably should be considerably heavier than that used in the formation of ordinary commercial briquets, such additional pressure having the important function of producing a dense mass of 10 heavy weight which successfully resists the entrance of moisture. This is highly important because moisture in the briquet renders very difficult the successful reconversion of the fuel into a combustible powder by my 15 process.

The pulverizing and briquetting operations above described may be performed at the coal mine or at the coal yard, or at any other suitable point remote from the point 20 where the fuel is to be burned, and the blocks or briquets thus prepared may be easily transported to the point of use and stored in a bin. There is no liability of the fuel in this condition exploding, and, therefore, 25 it is perfectly safe to store it in a home, apartment house, or any other desired place.

In burning the fuel, I may employ any 30 of the well-known types of pulverized fuel burners, and I take the blocks or briquets and, by suitable apparatus, scrape or shave or abrade the fuel from the blocks in pulverized form at the proper rate required by the burner. The apparatus for scraping or 35 shaving or abrading the fuel from the blocks should be of such a nature as to reduce the fuel to the proper degree of fineness for perfect combustion, and this pulverized fuel is then immediately introduced into a blast 40 of air which conveys it to the burner in the usual manner.

The advantage in this method of preparing 45 the fuel for the burner is that the fuel throughout the blocks or briquets will be of uniform density or structure so that as the pulverized fuel is removed from the blocks it will be uniform in character and also may be removed at a uniform rate.

One advantage in subjecting the blocks, 50 in the briquetting operation, to a sufficient pressure to bring the oil in the fuel to the surface of the particles is that this oil then acts more or less as a lubricant for the apparatus which scrapes or shaves off the par-

ticles, thereby lessening the wear on this apparatus. 55

Having thus described my invention, what I claim is:

1. The method of preparing solid fuel for burning as pulverized fuel which consists in 60 initially pulverizing the fuel, then compressing the pulverized fuel into briquets, and then removing said pulverized fuel from the surfaces of the briquets and immediately delivering the same to a burner. 65

2. The method of preparing solid fuel for burning as pulverized fuel which consists in initially pulverizing the fuel, then mixing the pulverized fuel with a binder and compressing it into briquets, then removing the 70 fuel from the surface of the briquets in a pulverized form suitable for combustion and immediately delivering the thus pulverized fuel into the burner.

3. The method of preparing solid fuel for 75 burning as a pulverized fuel which consists in initially pulverizing the fuel, then mixing the fuel with a binder and compressing it into a briquet, then removing the pulverized fuel from the surface of the briquet at 80 a properly regulated rate depending upon the requirements of the burner, and then immediately delivering the pulverized fuel into a current of air which conveys it to the burner. 85

4. The method of preparing coal for burning in pulverized form which consists in initially pulverizing the coal, mixing the coal with a binder and compressing it into 90 briquets, and then removing the fuel from the surface of the briquets in pulverized form and introducing it into a current of air which immediately delivers the fuel to the burner.

5. A briquet made from substantially dry 95 solid fuel pulverized to a uniform fineness and heavily compressed to form a dense substantially moisture-free and moisture-resisting mass capable of having a powder of uniform fineness scraped or abraded from its surface. 100

6. A briquet made from soft coal which has been reduced to pulverized form, mixed with a binder, and compressed with sufficient pressure to bring the oil in the particles of coal to the surface of these particles. 105

In testimony whereof, I hereunto affix my signature.

LEE B. GREEN.